

# UNITED STATES PATENT OFFICE.

WILLIAM W. NEUER, OF WILKES-BARRE, PENNSYLVANIA.

## PREVENTING DISCOLORATION OF BURNED BRICK.

SPECIFICATION forming part of Letters Patent No. 340,609, dated April 27, 1886.

Application filed February 5, 1886. Serial No. 190,947. (No specimens.)

*To all whom it may concern:*

Be it known that I, WILLIAM W. NEUER, a citizen of the United States, residing at Wilkes-Barre, in the county of Luzerne and State of Pennsylvania, have invented a new and useful Composition of Matter to be used for Preventing Discoloration of Burned Brick and Terra-Cotta and for Preserving the Brick and Terra-Cotta, of which the following is a specification.

My composition consists of the following ingredients, combined in the proportions stated, viz:

First. Vegetable oil, ten gallons; petroleum oil, ten gallons, this mixture to be applied to the surface of brick or terra-cotta as a first coating, (or application.)

Second. Melted beeswax, one gallon; turpentine, one gallon; vegetable oil, eighteen gallons, these ingredients to be thoroughly mixed and applied to the brick or terra cotta as a second application (or coating.)

Previous to applying the ingredients above described the bricks, terra-cotta, or other materials are first cleaned by using diluted nitric acid, (one part of the acid to four parts of water,) and such application should be made with a stiff brush. The acid is then washed off with clean water and the bricks or other material thoroughly dried. After this drying has been properly completed the compound of vegetable oil and petroleum is applied with a bristle brush, as much being used as the brick or material will thoroughly absorb, and the composition is then allowed to thoroughly dry. The second composition—beeswax, vege-

table oil, and turpentine—is then applied with a brush and allowed to properly dry. Thus the pores of the bricks or other material are thoroughly filled up, and the surface is completely protected against contact with moisture or other discoloring or injurious substances.

What I claim, and desire to secure by Letters Patent of the United States, is—

1. The herein-described composition of matter to be used for preventing the discoloration and preserving brick, &c., and terra-cotta, consisting of vegetable oil, petroleum-oil, beeswax, and turpentine.

2. The method of preventing discoloration of bricks, &c., the same consisting in first applying petroleum and vegetable oil to fill up the pores and interstices of the material and subsequently applying beeswax, vegetable oil, and turpentine to protect the surface of the material, substantially as described.

3. The method of preventing discoloration of bricks, &c., the same consisting in first applying to the bricks or other material a cleansing compound of nitric acid and water, then applying a composition of petroleum and vegetable oil to fill the pores of the material, and finally applying a composition of beeswax, vegetable oil, and turpentine to protect the surface of the material, substantially as set forth.

WILLIAM W. NEUER.

In presence of—

STANLEY W. WALKER,  
CHAS. A. ZIEGLER.